

## UNITED STATES PATENT OFFICE

JOHN LEATHART HANKEY, OF SALE, MANCHESTER, ENGLAND

## TREATING TEXTILE MATERIAL WITH CHROMIUM

No Drawing. Application filed April 4, 1929, Serial No. 352,615, and in Great Britain April 30, 1928.

It is well known that it is difficult to obtain a heavy chromium mordant on cotton. Thus, in a "Manual of Dyeing," by Knecht, Rawson & Löwenthal, 7th edition, 1922, p. 252, it is pointed out that: "It is difficult to impregnate the vegetable fibres with an amount of chromium salt sufficient to obtain a full shade . . . the demand for a good chromium mordant for the dyeing of cotton . . . has not been completely satisfied as yet."

Again, in the specification of British Patent No. 117,715 (1917), page 3, lines 27-28, after reference to the above passage in an earlier edition of Knecht, the following occurs: "As there has been no material improvement in the fixation of chromium mordants since, the problem remains unsolved." The new invention covered by the Patent No. 117,715 which has since lapsed is then described. It involves numerous operations and the fixing of the chromium on the fibre by relatively strong caustic lyes which, in actual practice, is a considerable drawback. Under the term "chromium oxide", I include the hydrated forms of chromium oxide usually referred to as chromium hydroxide and which may be represented by the formula  $\text{Cr}_2\text{O}_3 \cdot x\text{H}_2\text{O}$ ,  $x$  denoting zero or a positive number.

I have discovered a process whereby chromium may be fixed on the textile fibre efficiently and expeditiously without employment of strong caustic lye. To the best of my knowledge and belief by means of my invention chromium can be fixed on vegetable fibre in larger quantities than have hitherto been possible. On such heavily mordanted fibre very full and deep shades of alizarine and other mordant colours may be dyed.

I have further discovered that by fixing on vegetable fibre a large amount of chromium such fibre can be rendered practically fireproof. I do not mention a limit as regards the amount of chromium which must be fixed for this purpose. This will vary with the degree of fireproofing required, but as an example it may be stated that a cotton fabric having on the fibre fixed chromium equivalent to 28-30%  $\text{Cr}_2(\text{OH})_6 \cdot 4\text{H}_2\text{O}$  is

highly fireproof. A great advantage of this method of fireproofing over that depending on the use of soluble bodies such as ammonium sulphate, ammonium phosphate, sodium tungstate, borax, boracic acid and the like is that the fireproof quality of fabric treated by my process is not removed by wetting or washing. Of course, if desired, the chromium treatment may be followed by treatment with a water-soluble fireproofing body or bodies such as those mentioned above.

By means of my invention the feel and handle of cotton fabric can be modified and improved, and other advantages obtained.

My process consists in treating textile material with mixed solutions of a chromate of an alkali metal, preferably sodium chromate, and of a sulphoxylate of an alkali metal, such as are known in commerce under the names Formosul, Rongalite, Hydralite, Britulite, and the like.

I am aware that in the "Principles and Practice of Textile Printing," by Knecht and Fothergill, 1924, p. 213, there is described a process of mordanting calico by means of sodium bichromate neutralized with ammonia (which I term sodium-ammonium chromate) and formosul and I make no claim to such a process. The sodium-ammonium chromate formosul mixture referred to on which the process depends is unstable and within a short time of mixing, say an hour or less, has deposited appreciable quantities of a brown insoluble chromium compound. If filtered off, the deposition begins afresh, and, for this reason alone, the process can possess little practical interest. Material padded with this mixture and aged emerges from the age a brownish-olive colour, pointing to incompletely reduced chromium compound.

Furthermore, sodium-ammonium chromate is considerably less soluble than is sodium chromate and a saturated solution of sodium-ammonium chromate contains a much smaller equivalent of chromium in unit volume than does a saturated solution of sodium chromate; consequently the use of this latter solution permits of the blending of a padding liquor with a higher chromium

content than when sodium-ammonium chromate is employed and for this reason it can be caused to deposit a higher percentage of chromium on the fibre.

- 5 Again, a highly concentrated sodium-ammonium chromate formosul mixture is considerably less stable than a highly concentrated sodium chromate-formosul mixture in spite of the fact that the latter is the richer 70 in chromium. Thus a saturated solution of sodium-ammonium chromate at 18-20° C. possesses the specific gravity of about 60° Twaddell, and is approximately equivalent 75 in chromium content to 24-25 parts sodium bichromate in 100 parts by volume of solution, while a saturated solution of sodium chromate at the same temperature has sp. gr. of about 98° Tw. and is equivalent in chromium content to about 60 parts of sodium bichromate per 100 parts by volume of solution. On mixing 5 cc. of sodium-ammonium 80 chromate solution 60° Tw. with 10 cc. formosul 60° Tw., there is an appreciable evolution of heat, the liquor becomes quickly green and in about seven hours or less, at ordinary temperature, it will usually have turned into a solid gel of chromium hydrate. When quantities of 200-300 cc. are mixed, this change into gel may be immediate. On the other hand, by mixing 5 and 10 cc. respectively 85 of sodium chromate solution of 98° Tw. and formosul solution of 60° Tw., the temperature rises but slightly, the solution assumes an olive colour, and, if poured onto a filter paper, is yellow. It remains without solidifying into chromium gel for one to three days or more. It is quite easy to mix 200-300 cc. of concentrated sodium chromate and 90 formosul solutions without fear of premature gel formation. It will thus be seen that the process described by Knecht and Fothergill and the process of this specification are quite 95 distinct.

The following example illustrates my invention, which, however, is not confined to this example.

#### *Solution A*

Dissolve 600 g. sodium bichromate in 250 cc. hot water. Add 370 cc. caustic soda lye 75° Tw. Dilute the whole with water to one litre.

This gives a solution of 98-100° Tw. at 20-22° C.

#### *Solution B*

Dissolve 500 g. formosul in 620 cc. hot water and cool. This gives a solution of about 60° Tw. at 20° C.

To two parts by volume of Solution B gradually add, while stirring, one part by volume of Solution A. (In bulk work it may be desirable, though not essential to immerse the mixing vessel in cold water to prevent undesirable local rises of temperature.)

Pad dry bleached cotton fabric with this mixture and mangle so as to leave about 110% of liquor in the fabric. Without drying, age in moist steam at 100° C. for from 1/2-1 minute or longer according to the thickness of 70 fabric. If the steam is sufficiently moist, reduction is very quick. The fabric should come from the ager of a blue green (duck egg) colour. Rinse in hot or boiling water and dry. If it is necessary to remove all 75 alkali from the fabric, give a rinse in dilute acetic acid followed by a hot water rinse. According to the amount of chromium it is desired to incorporate with the fibre, the process may be repeated two, three or more times; 80 or if less chromium is required on the fabric, a more dilute padding mixture may be used, but in this case it is advisable to increase the relative proportion of formosul.

When the padding and steaming process 85 is to be repeated in order to incorporate additional chromium with the fibre, it is desirable that an acid rinse should be given after the material leaves the ager and instead of following this by a plain water rinse, there may 90 be added to the last water some wetting-out agent, e. g., such as may be obtained by the condensation with hydrocarbons of alcohols as propyl or butyl alcohol followed by sulphonation. The material is dried with the 95 wetting-out liquor adhering. Provided the wetting-out agent is of such a nature as not to form objectionable precipitates with the chromium padding liquor, its presence will 100 facilitate the penetration of the latter into the material. Another method of facilitating penetration during the second padding is to secure that after padding, ageing and rinsing, the material is only about three-quarters dried up, that is to say, it leaves the "tins" 105 or other drying apparatus with a slight amount of moisture left in it. Such procedure, however, is not essential, but merely a possible convenience, and after the first padding, ageing and rinsing, the material 110 may be dried up in the usual manner preparatory to further padding, if this is preferred.

The padding solution can be made still more stable by the addition of small quantities of caustic soda, glucose or glycerine, either 115 alone or in admixture, but excess must be avoided or the precipitation and fixation of chromium on the fibre may be hindered or even prevented. Also, lower temperatures than 100° C. may be used in the ager, provided sufficient time be given and the atmosphere remain sufficiently moist.

It is thought that the chromium is fixed in a form that may be represented by the formula  $\text{Cr}_2(\text{OH})_6 \cdot 4\text{H}_2\text{O}$ . As a guide, it 125 may be stated that a bleached cloth taken once through the aforementioned padding mixture and aged as directed retained chromium on the fibre equivalent to 13.1%  $\text{Cr}_2(\text{OH})_6 \cdot 4\text{H}_2\text{O}$ , which is equivalent to an 130

increase in weight of the original cloth of 15%. When the operation was repeated twice, making three times in all through the padding liquor, the chromium on the fibre was 5 equivalent to 28%  $\text{Cr}_2(\text{OH})_6 \cdot 4\text{H}_2\text{O}$ , which is equivalent to an increase of 39% on the original weight of the fabric.

The process can be applied to cotton, artificial silk, jute, linen, half-wool, natural 10 silk and tussah silk and other fibres, whether as loose material, yarn, cloth, etc.

What I claim and desire to secure by Letters Patent is:—

1. The process of fixing chromium on textile fibre which consists in treating such fibre with a mixture consisting of a chromate of an alkali metal and a sulphoxylate of an alkali metal, and ageing.

2. The process of fixing chromium on vegetable fibre which consists in treating such fibre with a mixture consisting of a chromate of an alkali metal and a sulphoxylate of an alkali metal, and ageing.

3. The process of fixing chromium on cotton fibre which consists in treating such fibre with a mixture consisting of a chromate of an alkali metal and sulphoxylate of an alkali metal, and ageing.

4. The process of fixing chromium on textile fibre which consists in treating such fibre with a mixture consisting of sodium chromate and sodium sulphoxylate, and ageing.

5. The process of fixing chromium on vegetable fibre which consists in treating such fibre with a mixture consisting of a sodium chromate and sodium sulphoxylate, and ageing.

6. The process of fixing chromium on cotton fibre which consists in treating such fibre with a mixture consisting of sodium chromate and sodium sulphoxylate, and ageing.

7. The process of fixing chromium on vegetable fibre in quantity sufficient to make it substantially fire-proof, which consists in impregnating it once or more than once with a mixture consisting of solutions of sodium chromate of about 100° Twaddell and of commercial sodium sulphoxylate of about 60° Twaddell, and ageing after each impregnation.

In testimony whereof, I affix my signature.  
JOHN LEATHART HANKEY.